

1

2,882,176

CELLULOSE ACETATE FIBERS CONTAINING  
NICKEL CARBONATE

James M. Straley and Raymond C. Harris, Kingsport, Tenn., assignors to Eastman Kodak Company, Rochester, N.Y., a corporation of New Jersey

No Drawing. Application January 30, 1957  
Serial No. 637,083

5 Claims. (Cl. 106—194)

This invention relates to cellulose acetate fibers of improved dyeing properties and to a method of producing said fibers. In a specific aspect this invention relates to cellulose acetate fibers containing a nickel salt of an organic acid, said fibers being capable of dyeing with a metallizable dye.

It is known in the art that compounds of metals such as nickel, chromium, cobalt and the like, react with certain dyes to produce stable colored metal complexes known as metallized dyes. Such dyes have been employed in the dyeing of cellulose acetate fibers. The metallized dye can be prepared by reacting the non-metallized dye with a suitable metal salt and the resulting metallized dye can then be used for dyeing cellulose acetate fibers. Alternatively, the cellulose acetate fibers can be dyed with the non-metallized dye and metallization of the dye can be effected on the fiber by reaction with a suitable metal salt. In either event, metallization of the dye is effected in a separate step or operation.

It is an object of this invention to provide a method for dyeing cellulose acetate fibers with non-metallized dyes wherein metallization of the dye is effected during the dyeing operation and without the necessity of a separate metallization step in the process. It is a further object of this invention to provide cellulose acetate fibers containing a metal salt such that during the dyeing of the fiber with a non-metallized dye, metallization of the dye is actually carried out.

In accordance with this invention, it has been found that addition of nickel carbonate to the cellulose acetate prior to dyeing of the cellulose acetate with a non-metallized metallizable dye makes it possible to dye the cellulose fiber and at the same time effect metallization of the dye on the fiber. The presence of the nickel carbonate on the cellulose acetate fiber presents several advantages. For example, the nickel carbonate causes no deacetylation of the cellulose acetate similar to that which can result when other metallic salts are used. Secondly, the low molecular weight of the nickel carbonate permits the introduction of a sufficient amount of metal into the fiber to effect metallization of the dye with a minimum of color being obtained from the nickel carbonate. Also the use of nickel carbonate makes it unnecessary to load up the fiber with sufficient foreign material to cause deterioration of the textile properties of the garment or fabric.

In practicing this invention, nickel carbonate is added to cellulose acetate at any time prior to its being spun into fiber. Thus, nickel carbonate can be added to melted cellulose acetate in a finely-divided state prior to the spinning of the melted cellulose acetate into fiber. Alternatively, finely-divided nickel carbonate can be mixed with granulated or powdered cellulose acetate prior to its being spun into fiber, either by a solution-spinning procedure or by a melt-spinning procedure. If solution spinning is employed, cellulose acetate can be dissolved in a

2

suitable solvent and nickel carbonate added to the solution prior to the spinning of the fiber.

An important feature of this invention is the use of a finely-divided pigment as a support for the nickel carbonate. Actually, the nickel carbonate can be used alone in practicing this invention, but good results can also be obtained when the nickel carbonate is deposited on a fine pigment that has an active surface or a porous structure prior to addition and incorporation in the cellulose acetate. The pigment prevents coagulation of the nickel carbonate during the processing of the cellulose acetate and it also tends to increase the exposed area of the nickel carbonate. In general, the pigment should have a particle size less than about 3 microns and preferably less than 0.5 micron. Suitable pigments that can be used are silica gel, activated alumina, ultra-fine calcium carbonate, magnesium carbonate, magnesium oxide, calcium silicate and magnesium silicate. The ultra-fine precipitated calcium carbonates are particularly suitable for use in practicing this invention.

Prior to incorporating the nickel carbonate in the cellulose acetate, it is preferable to grind the nickel carbonate to the desired particle size. The grinding or milling of the nickel carbonate can be carried out either with or without water and if any pigment, such as calcium carbonate, is employed, the pigment can be ground or milled along with the nickel carbonate. After grinding, the nickel carbonate can then be dried by suitable heating and it is ready for addition to the cellulose acetate. The amount of nickel carbonate that is employed is ordinarily within the range of 0.2 to 5 percent by weight of the cellulose acetate, preferably from 0.5 to 2 percent by weight.

After grinding, the nickel carbonate can be added to the cellulose acetate in accordance with this invention and in some instances, it may be found desirable to grind the mixture of nickel carbonate and cellulose acetate. The resulting intimate mixture can then be spun into fiber by a melt-spinning procedure or the mixture can be incorporated into a solvent and spun into a fiber from the resulting dope. In some instances, it may be desirable to incorporate a relatively high percentage of the nickel carbonate into the cellulose acetate and the resulting mixture can then serve as a concentrate or stock which can be diluted subsequently with additional cellulose acetate to obtain any desired concentration of nickel carbonate in the cellulose acetate.

The cellulose acetate that is employed to practice this invention can be prepared by any of the known procedures. For example, cellulose in the form of purified chemical cotton or wood pulp can be given a preliminary treatment with acetic acid. The mass of cellulose wet with acetic acid is then mixed with measured proportions of acetic anhydride catalyst, such as sulfuric acid, and solvent, such as methylene chloride. The resulting mixture is then agitated with suitable temperature control and the acetylating reaction converts the fibrous cellulose to a clear solution of cellulose triacetate. If desired, the cellulose triacetate can be recovered and employed in practicing this invention. However, many types of cellulose acetate are not in the triester form and the desired degree of acetylation is reached by a hydrolysis reaction induced by adding water and hydrolyzing agent to the triacetate dope with agitation and treatment to drive the reaction to the stage desired. The catalyst is then removed and the charge is precipitated into water followed by thorough purification procedures. The purified cellulose acetate is then dewatered and dried, placing it in a form useful for the practice of this invention.

70 The cellulose acetate employed in this invention can have a degree of acetylation ranging from about 50 per-

cent up to nearly 62.5 percent with a viscosity ranging from about 1 to 250 seconds. The viscosity can be measured by the time of fall of a steel ball through 10 inches of a 20 percent by weight solution of cellulose acetate dissolved in a 90:10 acetone:ethanol solution at 25° C.

The cellulose acetate containing nickel carbonate prepared in accordance with this invention can be employed to manufacture fibers or yarn in accordance with any of the known procedures. One of the more common methods for preparing cellulose acetate fibers or yarn involves a dry spinning process using an acetone solution. Concentrated acetone solutions of cellulose acetate are forced through spinnerets to form filaments which are cured by circulated air. The filaments or fibers are then gathered and passed over guide rolls to apply controlled twisting and stretching. If desired, a wet spinning procedure can also be used to form the cellulose acetate fibers or filaments. In such a process, the cellulose acetate containing nickel carbonate is dissolved in either acetic acid or chloroform solutions and spun into a precipitating liquid. Alternatively, a melt-spinning procedure can be used and in such a process the cellulose acetate is heated to a molten form and spun at the relatively high temperature into the desired filaments. The lower acetyl forms of cellulose acetate are more readily soluble in the common solvents and for that reason are quite adaptable to the wet and dry spinning procedures. The higher acetyl types of cellulose acetate are comparatively insoluble in the more common solvents and for that reason this form of cellulose acetate does not lend itself to use in the wet and dry spinning processes.

After being spun, the cellulose acetate fiber or filament containing nickel carbonate can be easily dyed with any of the dyes known to chelate or mordant with nickel. Among the dyes that can be used are those described in U. S. Patents 2,641,602 and 2,651,641. These dyes have the structural formulas:



wherein R is a phenylethyl alcohol nucleus, and



wherein A is a monocyclic benzene nucleus containing a



group wherein R represents hydrogen, methyl or ethyl.

The above dyes are representative of the compounds that can be used to chelate with the nickel carbonate in the cellulose acetate fibers of this invention. Other suitable dyes are described in the following copending applications:

- Straley and Fisher, Serial No. 458,262, filed September 24, 1954  
 Straley and Giles, Serial No. 466,955, filed November 4, 1954  
 5 Straley and Wallace, Serial No. 498,112, filed March 30, 1955

Those dyes known to chelate with nickel are employed to color cellulose acetate fibers in a manner similar to that employed by those skilled in this art heretofore.

*Example 1*

50 g. of nickel carbonate and 10,000 g. of a 5 percent solution of cellulose acetate in acetone are ground for 2.5 hours in a Szegvari Attritor. The resulting dope, filtered from the balls used, is adjusted with acetone and cellulose acetate to a dope suitable for spinning and containing 2,450 g. total of cellulose acetate. This dope is then spun into filaments.

- 20 *Example 2*  
 A fabric knitted from the filaments produced in Example 1 was well-scoured and then dyed in a strength of 4 percent with the dye having the formula:



30 
  
 at 80° C. There resulted a beautiful red dyeing of good light-and-wash fastness.

35 We claim:

1. In a process for producing a cellulose acetate fiber capable of being colored with a metallizable dye, the improvement which comprises incorporating nickel carbonate in the cellulose acetate from which the fiber is formed in an amount within the range of 0.2 to 5 percent by weight of the cellulose acetate prior to formation of said fiber.

2. A process according to claim 1 wherein the nickel carbonate is incorporated in an amount within the range of 0.5 to 2 percent by weight of the cellulose acetate.

3. A process according to claim 1 wherein the nickel carbonate is incorporated in the solution containing the cellulose acetate from which the fiber is formed.

4. As a new composition of matter, a cellulose acetate fiber capable of being colored with a metallizable dye, said fiber containing from 0.2 to 5 percent by weight of nickel carbonate.

5. As a new composition of matter, a cellulose acetate fiber capable of being colored with a metallizable dye, said fiber containing from 0.5 to 2 percent by weight of nickel carbonate.

References Cited in the file of this patent

UNITED STATES PATENTS

- 60 1,871,470 Rivat et al. \_\_\_\_\_ Aug. 16, 1932  
 2,052,557 Dreyfus \_\_\_\_\_ Sept. 1, 1936  
 2,052,558 Dreyfus \_\_\_\_\_ Sept. 1, 1936  
 2,206,278 Dreyfus \_\_\_\_\_ July 2, 1940

FOREIGN PATENTS

- 65 631,765 Great Britain \_\_\_\_\_ Nov. 19, 1949

UNITED STATES PATENT OFFICE  
CERTIFICATE OF CORRECTION

April 14, 1959

Patent No. 2,882,176

James M. Straley et al.

It is hereby certified that error appears in the printed specification of the above numbered patent requiring correction and that the said Letters Patent should read as corrected below.

Column 3, lines 44 and 45, lower left-hand portion of the formula,  
for

$\text{NH}_2$  read  $\text{NO}_2$

Signed and sealed this 1st day of September 1959.

(SEAL)

Attest:

KARL H. AXLINE

Attesting Officer

ROBERT C. WATSON  
Commissioner of Patents